

July 31, 1928.

1,678,718

DE WITT C. AMERINE

METHOD OF WASHING COOKED STRAW

Filed June 9, 1926



Inventor  
De Witt C. Amerine

By

*Stanley & Sonnen*

Attorney's

Patented July 31, 1928.

## UNITED STATES PATENT OFFICE.

DE WITT C. AMERINE, OF VINCENNES, INDIANA.

## METHOD OF WASHING COOKED STRAW.

Application filed June 9, 1926. Serial No. 114,700.

In the method heretofore employed, straw of all kinds has been placed in a globe rotary boiler and cooked under various steam pressures, the straw being saturated with a 5 solution of lime water which has a tendency during the cooking period of softening the straw to a point where the fibers could be separated in the next operation in manufacturing, which is the beater room. All 10 beater rooms where straw board or paper is manufactured are equipped with beaters of various makes and the beating engine itself is equipped with washing apparatus of the rotary or circular type and a method 15 was practised for some time of washing cooked straw with a solution of lime used for softening purposes. However, there is now in use a new method of softening straw in a rotary for the manufacture of strawboard 20 or paper by using lime sulphur, it being a patented process which has been developed by the paper mill laboratories, but lime sulphur, acts very differently from lime water and the washing arrangement which 25 operated entirely satisfactory for the purpose intended with the solution used is not adequate where lime sulphur is used in the manufacture of strawboard or paper, for the reason that if the stock was not properly 30 washed, in passing to the next step in its manufacture, which is the paper machine, this lime sulphur would rise to the surface of the sheet on the dryers and form a crust or case hardening which prevented the quick 35 movement of moisture from the sheet and with a given number of dryers to produce a given amount of tonnage it was very soon discovered that the new chemical would reduce production to a point that would 40 make the operation of the entire mill a losing venture.

The object of the invention is to overcome the difficulty that heretofore existed with the use of lime sulphur in the manufacture of 45 strawboard or paper.

Fig. 1 is a vertical sectional view through the rotary showing the connections to the steam pipe and pump in full lines. Fig. 2 is a detail sectional view of the coupling for 50 the steam and water pipe. Fig. 3 is a vertical view on the lines 3—3 of Fig. 1.

Like letters of reference indicate like parts throughout the different views.

The drum is indicated by 1. The drum 55 has manholes 2 and 3 and the cooked straw is inserted through these manholes. It is

to be understood that in the operation of these machines the rotaries usually are capable of holding 7½ tons of straw and this straw must be inserted at frequent intervals 60 until the capacity of the rotary is reached. It is usual to insert about one-third of the amount at the beginning of the operation and after the rotary has been operated for some period of time additional straw is inserted and this continues until the capacity 65 of the rotary is reached, but toward the end of the normal operation of this rotary the straw is compacted sufficiently so that it will fill only part of the rotary and consequently 70 during the rotary movement this compacted straw will be thrown from one part of the rotary to the opposite part thereof. In order to adapt the rotary for the new method employed therein, I found it desirable to 75 use a perforated plate 4 which is secured to the rotary near one end thereof as shown in Fig. 1. This plate may be inserted in section through the manhole or it may be built in the rotary when same is constructed, but it 80 is preferably shown riveted to the sides of the rotary and is so placed that there is a space 5 formed between the plate and the end of the rotary. This plate is shown at 85 the right hand side of Fig. 1. The perforations 6 are of such number and arranged in such a way that they will permit of the escape of the water hereinafter referred to and they co-operate with the movement of the compacted straw to permit the escape 90 of water. The rotary 1 is supported on bearings 7 and 8 in any usual and ordinary way and same is rotated in the regular way which is a series of gearing, one of which 95 is indicated by 9, which reduces the rotary to a speed for practical operation of same.

There is also shown a pipe connection for the steam and water at the left hand side of Fig. 1. This pipe is marked 10 and is secured to the inside of the rotary by clips 11 100 and the lower end of the pipe extends to a point near one of the manholes, it being apparent that the manholes are off set one from the other. This pipe terminates as shown in Fig. 2 in a socket 12 formed on 105 the end of pipe 13 which is a stationary pipe extending from the water and steam connection. The pipe 10 rotates with the rotary and there is formed an ordinary loose connection between the pipe 12 and the pipe 10 110 as shown clearly in Fig. 2 which enables the pipe 10 to rotate independently of the pipe

13. There is also shown means such as glands 14 for protecting the device from the escape of steam.

The water pump is indicated by 15 and the pipe 16 extends from the pump to the pipe 13. There is also shown a pipe 17 which is connected with any ordinary steam device.

In the beginning of the operation the water connections are shut off by valves 18 and 19, the valve 19 being located on the outlet pipe 20 which also extends within the rotary by means of the connecting pipe 21. Pipe 21 is securely fastened to the outer section or half of steam joint or coupling 22, which is connected on outside end of journal, and remains in a fixed position inside of rotary. Coupling or steam joint 22 is similar to the coupling or steam joint shown in Figure 2 which enables pipe 21 to remain stationary and is for the same purpose as pipe 20, both for the purpose of discharge and as appears clearly in Fig. 1, the lower end of the pipe 21 terminates near the lower edge of plate 4 and this is arranged so as to insure the water and lime sulphur siphoning out of the rotary at the end of the operation as will be more fully explained hereafter.

The normal operation of this apparatus and method is to insert with the straw or through the manhole after the straw has been first inserted, a sufficient amount of lime sulphur to cause the straw when cooked to be sufficiently softened, after a period of 8 or 10 hours, to make it suitable for forming straw board or paper. This lime sulphur remains in the rotary until the straw itself is about to be removed; and the steam connections are kept open so that during the period of 8 hours the straw is kept within the rotary under about 40 pounds steam pressure and this with the lime sulphur causes the straw to be sufficiently softened for its intended purpose. After this has been accomplished the valve 23 shown in the steam pipe 17, is operated to shut off the steam connection and the valves 18 and 19 are then opened and the pump or other mechanism started to pump water into the rotary.

Under the old method or the general practice immediately after the 8 or 10 hour cooking period the steam is shut off the rotary, the rotary stopped and a pipe line is connected with a blow off valve which is set generally about 2 feet in front or back of the head or manhole; after this blow off line is arranged the operator opens blow off valve and in this method the pressure is reduced to where the manhead can be taken out and the contents of rotary dumped into what is known as a stock room, but with the new apparatus the time lost during the blow off period which is about 45 minutes is now used as washing time or for washing purposes.

I have described in the above paragraph

various valves and pipe lines for the handling of steam or water and the relieving of the water during the washing process and this washing process is continued until the consistency of the chemical, which slows the stock through the mill, is reduced to where the present washing arrangement in the beater room is sufficient to clear the stock so that the production on machine is not interfered with.

After carrying on this washing arrangement in the rotary for a sufficient period of time the pump is shut down and valve 18 is closed, valve 19 is left open until the liquor or solution is siphoned or until the vacuum is broken on the end of pipe 21. The rotary is then stopped, manhead taken out, and the discharging of contents of rotary is carried on in the usual manner. This washing operation in rotary is not a loss of time, it has been going on during the period which otherwise would have been consumed in blowing down pressure which would permit the operator to get out manhead and get the rotary up to the present point above described and this produces a stock which is now in shape to be handled without loss of production in other departments of a mill.

It is usual in straw board or paper plants to operate the rotary room during the day time, the balance of the mill is a 24 hour operation. The night period of rotary room operation is the time consumed in cooking and dumping, all mills having rotary capacity enough to carry on the operation as stated above.

It is further to be understood that the water is forced into the rotary immediately after the cooking operation is completed and it is therefore important to use a pump or other means of sufficient size and power such that the water will be forced into the rotary against 40 pounds steam pressure or thereabout.

Having described the invention, I claim as follows:

1. The method of treating straw for straw boards or papers by first rotating same in a closed vessel with a lime sulphur in the presence of steam under pressure and thereafter continuing the rotation of said rotary with a restricted outlet in said vessel, and applying water against the pressure of the steam held in said vessel, whereby the water will flow through said vessel, reducing the pressure of the steam and removing from the vessel a portion of the said solution.

2. The method of treating straw for use in making straw board or paper by rotating same in a closed vessel for a predetermined period of time having therein a lime sulphur solution with steam applied to said closed vessel under pressure and after a predetermined period of rotation shutting off the application of steam and then applying water

against the pressure of the entrapped steam through said vessel into a restricted outlet for said vessel whereby the pressure of the steam will be reduced while the solution is being likewise diluted and partially removed from said vessel.

3. The method of softening straw for straw board or paper purposes by first rotating same in the presence of steam under pressure and a lime sulphur solution for a predetermined period of time and thereafter continuing the rotation of same with a flow of water passing through said straw, simultaneously reducing the pressure of the steam and diluting the solution whereby the straw will be made suitable for more profitable operation.

4. The method of treating straw for straw board or paper by first rotating same in a closed vessel with a chemical solution suitable for softening the straw in the presence of steam under pressure and thereafter continuing the rotation of said rotary with a restricted outlet in said vessel and applying

water against the pressure of the steam held in said vessel whereby the water will flow through same reducing the pressure of the steam and simultaneously removing from the vessel a portion of the said solution.

5. The method of treating straw by rotating same in a closed vessel with a chemical solution for softening the straw in the presence of steam maintained for a substantial period of time and thereafter subjecting same to a washing process by applying water against the pressure of the steam for a period of time amounting to only a fraction of the first mentioned period of time while continuing the rotation of said rotary with a restricted outlet in said vessel whereby the pressure of the steam will gradually be reduced and a portion of the solution be simultaneously removed from said vessel by a siphoning action.

In testimony whereof, I have hereunto set my hand this eighth day of May, 1926.

DE WITT C. AMERINE.